

B. PERRIS,  
METAL COATING FOR ARC LIGHT ELECTRODES.  
APPLICATION FILED OCT. 25, 1912.

1,148,189.

Patented July 27, 1915.



WITNESSES

*H.G. Grover*  
*C.W. vonbach*

INVENTOR  
BEN PERRIS

BY *Ira J. Adams*  
ATTORNEY

# UNITED STATES PATENT OFFICE.

BEN PERRIS, OF CLEVELAND, OHIO, ASSIGNOR TO NATIONAL CARBON COMPANY, OF CLEVELAND, OHIO, A CORPORATION OF NEW JERSEY.

## METAL COATING FOR ARC-LIGHT ELECTRODES.

1,148,189.

Specification of Letters Patent.

Patented July 27, 1915.

Application filed October 25, 1912. Serial No. 727,742.

To all whom it may concern:

Be it known that I, BEN PERRIS, a citizen of the United States, and a resident of Cleveland, in the county of Cuyahoga, in the State of Ohio, have invented new and useful Improvements in Metal Coatings for Arc-Light Electrodes, of which the following is a clear and exact description.

This invention relates to metal coatings for arc light electrodes.

One of the objects is to apply the metal coating in such a manner that it will not pull away from the electrode to cause spindling when burned in the lamp.

Another object is to prevent the coating from obscuring the light by protruding above the electrode end.

Other objects will appear in the appended description.

In the drawings the figure shows an electrode having a coating in accordance with my invention.

Some types of electric light carbons are plated with metal, usually copper, throughout the greater part of their length to decrease the resistance, or at the holder end to decrease the contact resistance. A metal

plate coating, such as electroplate, thin tube or other form has objectionable features

when used on an arc light carbon. The plate is liable to separate from the hot end of the electrode when burning and this causes spindling. Another objectionable feature is that the solid plating of metal re-

sists the action of the arc to a greater extent than does the carbon electrode. Conse-

quently it sometimes extends more or less above the electrode and obscures the light. This difficulty is met with, both when it is electroplated and when it is put on mechanically in the shape of a tube or other form.

I have found that if the coat is put on in the shape of a metal powder, none of the above mentioned difficulties are met with. A metal paint is first formed by mixing powdered copper, bronze or other metals with some matrix of varnish or other sizing which sets very hard at ordinary temperatures. This paint is applied to the carbons with a fine brush or the carbons may be dipped in it and the excess allowed to drain off. When the paint sets it adheres very firmly and furnishes a good conductor of electricity. Since the coating is not in the form of a continuous sheet, but exists in the form of a powder it does not pull away from the carbon nor extend above the burning end of the electrode. The metal particles become sweated to the carbon at the arcing end and always remain just below the burning point.

Having described my invention what I claim is:

An arc lamp electrode having a coating of metal powder secured to it by a binder.

In testimony whereof I have hereunto signed my name in the presence of two witnesses.

BEN PERRIS.

Witnesses:

I. J. ADAMS,  
G. H. BROWN.